

No. 776,474.

PATENTED NOV. 29, 1904.

R. KRON.

PROCESS OF PRODUCING YARN FROM MAGAZINE ROLLS OF SHORT FIBER MATERIAL IN A MOIST CONDITION.

APPLICATION FILED MAY 22, 1903.

NO MODEL.



Witnesses:-  
Henry Schmid  
George Baumg

Inventor:-  
Rudolf Kron  
by attorney  
Brown & Howard

## UNITED STATES PATENT OFFICE.

RUDOLF KRON, OF GOLZERN, GERMANY.

## PROCESS OF PRODUCING YARN FROM MAGAZINE-ROLLS OF SHORT-FIBER MATERIAL IN A MOIST CONDITION.

SPECIFICATION forming part of Letters Patent No. 776,474, dated November 29, 1904.

Original application filed December 6, 1902, Serial No. 134,201. Divided and this application filed May 22, 1903. Serial No. 158,260. (No specimens.)

*To all whom it may concern:*

Be it known that I, RUDOLF KRON, a citizen of the Republic of Switzerland, and a resident of Golzern, in the Kingdom of Saxony, in the 5 German Empire, have invented new and useful Improvements in Processes for the Production of Yarn from Magazine - Rolls of Short-Fiber Material in a Moist Condition, of which the following is a specification, reference being had to the accompanying drawings, 10 designed to show the magazine-roll employed in producing the desired result.

The present invention, which has been described in my application, Serial No. 134,201, 15 filed December 6, 1902, of which the present application is a division, has for its object a process for the production of yarn from magazine-rolls of short-fiber material in a moist condition; and it consists, first, in drawing 20 off separate one or more strips from a web composed of short-fiber material—as paper-pulp, cellulose, asbestos, silk, and the like—provided in a longitudinal direction with furrows a suitable distance apart and rolled up 25 in a moist condition, and, second, in twisting said strips in a moist condition on a spinning, 30 spooling, or twisting machine, one such strip being twisted singly or two or more being twisted together. For the purpose of producing yarn from magazine-rolls the endless 35 web of paper-pulp being still in a moist condition is provided by suitable means and before its rolling up with longitudinal furrows a suitable distance apart. The rolling off 40 from the magazine-roll takes place in the form of separate small strips by dividing the web along the longitudinal furrows formed in such web. This rolling or drawing off of small strips from the magazine-roll is possible only 45 if the web of paper-pulp is still in a moist condition. The web rolled up in a moist condition maintains or insures a sufficient moisture during weeks and months, so that magazine-rolls can be kept in stock.

For supplying the spinning, spooling, or twisting machines with the magazine - rolls

produced according to the process described above the rolls of a considerable width are divided, by means of cutting, sawing, and other mechanical means, in sections, and these 50 sections of the original roll are placed in a vertical, horizontal, or inclined position in front of the machine.

Figures 1 and 2 of the annexed drawings show in side view a section of a divided magazine-roll composed of a plurality of separate strips or strips divided by furrows, but adhering still together by a thin film. Such a section of a magazine-roll can be placed horizontally, and the single strips supplied to the 60 spinning, spooling, or twisting machine can be drawn off from the periphery of the magazine-roll, as shown in Fig. 1, or from the inner surface of the roll mentioned, as shown in Fig. 2, which shows part of the roll in section. Two or more of the sections of a magazine-roll can also be placed in front of the 65 spinning, spooling, or twisting machine in a vertical position, as shown in Figs. 3 and 4, Fig. 3 showing in front view part of a twisting-machine, and Fig. 4 a plan of same.

aa are two sections of a magazine-roll placed on a core b. The strips of the roll, still adhering together by a thin and narrow film, are drawn off from the rolls, as shown, and guided 75 to the stationary guide-pins c, set to change the course of the strips d, and spread them in lines diverging toward the rollers e. The strips d are thereafter guided to fliers g and bobbins f, which may be of similar construction to those in general use for spinning. By these fliers the strips d may be twisted singly, 80 as illustrated at the left of Fig. 3, or two or more together, as illustrated at the right of the same figure.

What I claim as my invention is—

The process herein described for the manufacturing of yarn from magazine - rolls of short-fiber material in a moist condition, said process consisting in rolling off separate—one 90 or more—strips from an endless web consisting of the short-fiber material furrowed in

the direction of its length at suitable intervals and rolled up in a moist condition and in twisting said moist strips in a spinning, spooling, or twisting machine in which said strips 5 may be twisted singly or two or more together.

In testimony that I claim the foregoing as

my invention I have signed my name, in presence of two witnesses, this 4th day of May, 1903.

RUDOLF KRON.

Witnesses:

RUDOLF SCHMIDT,  
PAUL ARRAS.